# EUROPEAN PATENT SPECIFICATION

(11) **EP 0 913 850 B1**
(45) Date of publication and mention of the grant of the patent: **10.05.2006**
(21) Application number: 98308817.0
(22) Date of filing: 28.10.1998
(51) Int. Cl.: H01J 1/30, H01J 9/02

(54) **Narrow titanium-containing wire, process for producing narrow titanium-containing wire, structure, and electron-emitting device**
Schmaler Titan enthaltender Draht, Verfahren zur Herstellung, Struktur, und elektronemittierende Vorrichtung
Fil étroit contenant du titane, procédé de fabrication, structure et dispositif émetteur d'électrons

(30) Priority: 30.10.1997 JP 29866297; 19.10.1998 JP 31393998
(43) Date of publication of application: 06.05.1999
(73) Proprietor: CANON KABUSHIKI KAISHA, Tokyo (JP)
(72) Inventor: Iwasaki, Tatsuya, Ohta-ku, Tokyo (JP); Den, Tohru, Ohta-ku, Tokyo (JP)
(74) Representative: Beresford, Keith Denis Lewis

(56) References cited:
- EP-A- 0 351 110
- EP-A- 0 364 964
- WO-A-95/07543
- WO-A-98/48456
- DE-A- 19 602 595
- US-A- 3 783 325
- US-A- 4 163 918
- US-A- 4 345 181
- US-A- 4 379 250
- US-A- 5 164 632
- US-A- 5 581 091
- ROUTKEVITCH D ET AL: "POROUS ANODIC ALUMINA TEMPLATES FOR ADVANCED NANOFABRICATION" 1997 , ELECTROCHEMICAL SOCIETY PROCEEDINGS, VOL. 97-7, PAGE(S) 350 - 357 XP002072447 * page 354, line 31 - line 41 *
- ROUTKEVITCH D ET AL: "NONLITHOGRAPHIC NANO-WIRE ARRAYS: FABRICATION, PHYSICS, AND DEVICE APPLICATIONS" October 1996 , IEEE TRANSACTIONS ON ELECTRON DEVICES, VOL. 43, NR. 10, PAGE(S) 1646 - 1658 XP002072446
- P.HOYER ET AL.: "ELECTRODEPOSITED NANOPOROUS TiO2 film by a two-step process from anodic porous alumina " JOURNAL OF MATERIALS SCIENCE LETTERS, vol. 15, 1996, pages 1228-1230, XP002091820
- PATENT ABSTRACTS OF JAPAN vol. 018, no. 345 (E-1571), 29 June 1994 & JP 06 089651 A (OSAKA PREFECTURE;OTHERS: 01), 29 March 1994

## Description

### BACKGROUND OF THE INVENTION

### Field of the Invention

The present invention relates to a narrow titanium- containing wire, a production process thereof, a nanostructure and an electron-emitting device, and more particularly to a narrow wire which can be widely used as a functional material or structural material for electron devices, microdevices and the like, in particular, as a functional material for photoelectric transducers, photo-catalytic devices, electron-emitting materials, narrow wires for micromachines, narrow wires for quantum effect devices, and the like, a production process thereof, a nanostructure comprising the narrow wire, and an electron-emitting device using the nanostructure. Related Background Art

Titanium and alloys thereof have heretofore been widely used as structural materials for aircraft, automobile, chemical equipment and the like because of their mechanical features that they are light-weight, strong and hard to be corroded. Besides, titanium and alloys thereof are also in use as medical materials because they are harmless to human bodies.

Recently, researches of solar cells, decomposition of injurious materials, antibacterial action, etc. have been being extensively made as applications of the photo-conductive properties, photocatalytic activity and the like of titanium oxide.

Besides, the application range of titanium materials extends to many fields such as vacuum getter materials, electron-emitting materials, metallic alloys for hydrogen storage and electrodes for various electron devices.

On the other hand, thin films, narrow wires, small dots and the like of metals and semiconductors may exhibit specific electrical, optical and/or chemical properties in some cases because the movement of electrons is restricted at smaller size of a certain characteristic length.

From this point of view, an interest in materials (nanostructures) having a structure minuter than 100 nm as functional materials is greatly increasing.

An example of a method for producing a nanostructure includes a production by semiconductor processing techniques including minute pattern writing techniques such as photolithography, electron beam exposure and X-ray diffraction exposure.

Besides such a production method, it is attempted to realize a novel nanostructure on the basis of a naturally formed regular structure, i.e., self-ordered structure. Since this technique has a possibility that a fine and special structure superior to those produced by the conventional methods may be produced, many researches are beginning to be carried out.

An example of the specific self-ordered nanostructure is an anodically oxidized aluminum film [see, for example, R. C. Furneaux, W. R. Rigby & A. P. Davidson, NATURE Vol. 337, p. 147 (1989)]. This anodically oxidized aluminum film (hereinafter called "porous alumina") is formed by anodically oxidizing an Al plate in an acid electrolyte. As illustrated in Fig. 6, its feature resides in that it has a specific geometric structure that narrow cylindrical pores (nanoholes) 14 as extremely fine as several nanometers to several hundreds nanometers in diameter are arranged at intervals of several nanometers to several hundreds nanometers in parallel with one another. These narrow cylindrical pores 14 have a high aspect ratio and are excellent in linearity and uniformity of sectional diameter.

Various applications are being attempted by using the specific geometric structure of such a porous alumina as a base. The detailed explanation thereof is found in Masuda [Masuda, KOTAI-BUTSURI (Solid-State Physics), 31, 493, 1996]. Techniques for filling a metal or semiconductor into narrow pores and techniques for taking a replica are typical, and various applications including coloring, magnetic recording media, EL light-emitting devices, electrochromic devices, optical devices, solar cells and gas sensors are attempted.

Further, applications to many fields such as quantum effect devices such as quantum wires and MIM (metal-insulator-metal) tunnel effect devices, and molecular sensors using nanoholes as chemical reaction sites are expected.

If such a nanostructure made with a highly functional material, i.e., titanium, is available, the nanostructure is expected to be utilized as a functional structure such as electron devices, microdevices, etc.

As an example where a nanostructure is produced by using a titanium material and controlling size and form, may be mentioned patterning of a thin film of the titanium material by semiconductor processing techniques including minute pattern writing techniques such as photolithography, electron beam exposure and X-ray diffraction exposure as described above. However, these techniques involve problems of poor yield and high cost of apparatus, and there is thus a demand for development of a simple method for producing a nanostructure with good reproducibility.

The method using the self-ordering phenomenon, particularly, the method using the porous alumina as a base is preferable to the method using such a semiconductor processing technique because it has a merit that a nanostructure can be easily produced over a large area under good control.

As an example where a titanium-containing nanostructure was produced by applying such a method, may be mentioned an example by Masuda et al., in which porous TiO₂ was formed by taking a replica of porous alumina with titanium oxide [Jpn. J. Appl. Phys., 31 L1775-L1777 (1992); and J. of Materials Sci. Lett., 15, 1228-1230 (1996)].

However, this method involves problems to be solved such as it must go through many complicated steps in the process of taking the replica, and the crystallinity of TiO₂ is poor since it is formed by electrodeposition.

On the other hand, it is often conducted to filling a metal or semiconductor into narrow pores of the porous alumina, thereby producing a nanostructure. Examples thereof include filling of Ni, Fe, Co. Cd or the like by an electrochemical method [see D. Al-Mawlawi et al., Mater. Res., 9, 1014 (1994); and Masuda et al., Hyomen-Gijutsu (Surface Techniques), Vol. 43, 798 (1992)], and melt introduction of In, Sn, Se, Te or the like [see C. A. Huber et al., SCIENCE, 263, 800 (1994)]. However, the filling of a Ti-containing material according to either method has not been reported from the reasons that the electrodeposition of Ti is not common, and that the Ti materials generally have a high melting point.

On the other hand, potassium titanate whiskers of the submicron size (0.2 to 1.0 µm in diameter, 5 to 60 µm in length) have been developed as applications to fiber reinforced plastics, fiber reinforced metals and fiber reinforced ceramics [Nihon-Kinzoku-Gakkai-shi (Journal of The Japan Institute of Metals), 58, 69-77 (1994)]. However, these materials are all powdery, and no technique for position-controlling and arranging them on a substrate have been known as yet. In order to expect specific electrical, optical and chemical properties as nanostructures, there is also the necessity of further narrowing them in size.

United States Patent No. 5,581,091 discloses nanoelectric devices suitable for use as diodes, transistors or other electronic components. These are prepared by electrolytically anodizing a metal substrate in sheet or foil form in an acid bath to deposit an oxide film having axially disposed micropores of substantially uniform diameter and substantially uniform depth. The thickness of the oxide film is greater than the depth of the micropores, so that an insulative layer of oxide film is provided at the bases of each micropore. Conductive material is deposited in the micropores to form nanowires contacting the oxide layer at the base of the micropores. Macrometal is then deposited over the ends of the nanowires for external electrical contact purposes.

United States Patent No. 5,164,632 discloses an electron emission element including an electrically insulating member made from an anodic oxidation film and having a plurality of pores extending between its upper and lower surfaces. An electron emission member is disposed in each pore. The emission member is made from a conductive material such as gold, and has a pointed end directed toward the upper end of the pore. An electrode is disposed around an upper portion of each pore and is separated from the electron emission member disposed in the pore.

### SUMMARY OF THE INVENTION

The present invention has been made in view of such various technical requirements as described above, and it is an object of the present invention to provide a process for producing a narrow titanium-containing wire, using titanium as a main material, particularly, a process for producing a narrow titanium-containing wire on a substrate.

Another object of the present invention is to provide a structure provided with narrow titanium-containing wires having a specific direction and a uniform diameter arranged at regular intervals on a substrate.

A further object of the present invention is to provide a high-performance electron-emitting device capable of emitting electrons in a greater amount.

The above objects can be achieved by the present invention described below.

According to the present invention, there is thus provided a process for producing a structure having narrow titanium-containing wires, comprising steps of:
(i) providing a structure comprising a substrate having a titanium-containing surface and thereon a porous layer having narrow pores reaching said titanium-containing surface; and
(ii) forming narrow titanium-containing wires projecting from said titanium-containing surface into the respective narrow pores by heat treatment under a specific atmosphere of the structure provided in step (i).

According to the present invention, there is also provided a structure comprising a substrate having a surface containing titanium, and narrow titanium-containing wires projecting from said titanium-containing surface, in a direction substantially vertical to the surface.

According to the present invention, there is still further provided an electron-emitting device comprising a structure, which comprises a substrate having a titanium-containing surface, a porous layer thereon having narrow pores reaching said titanium-containing surface, and narrow titanium-containing wires projecting from said titanium-containing surface respectively formed in the narrow pores; a counter electrode arranged in an opposing relation to the titanium-containing surface; and a means for applying a potential between the titanium-containing surface and the counter electrode.

According to the embodiments of the present invention, there can be realized a narrow titanium-containing wire and a titanium-containing nanostructure having a structure of a nanometer scale.

The nanostructure provided with the narrow titanium- containing wires according to the embodiment of the present invention can be widely applied as a functional material or structural material for various kinds of electron devices and microdevices, including photoelectric transducers, photocatalysts, quantum wires, MIM devices, electron-emitting devices and vacuum getter materials.

The narrow titanium-containing wires according to the embodiment of the present invention can also be used as a reinforcement for plastics and the like.

### BRIEF DESCRIPTION OF THE DRAWINGS

Figs. 1A, 1B, 1C and 1D conceptually illustrate examples of the form of a narrow titanium-containing wire according to the present invention, in which Fig. 1A illustrates the form like a strand, Fig. 1B illustrates the form like a column, Fig. 1C illustrates the form like a column the diameter of which successively varies, and Fig. 1D illustrates the form with a plurality of columns united.
Figs. 2A, 2B, 2C and 2D are conceptual cross-sectional views illustrating a production process of a nanostructure according to an embodiment of the present invention, in which Fig. 2A illustrates a step of providing a substrate with a titanium-containing film formed on a base, Fig. 2B illustrates a step of forming an Al-containing film on the substrate, Fig. 2C illustrates a step of anodizing the Al-containing film to form a porous alumina, and Fig. 2D illustrates a step of forming narrow titanium-containing wires in the respective narrow pores of the porous alumina.
Figs. 3A, 3B, 3C and 3D conceptually illustrate examples of a nanostructure to which the narrow titanium- containing wire according to the present invention is applied, in which Fig. 3A illustrates a nanostructure provided with the narrow titanium-containing wires arranged in the direction substantially vertical to a substrate, and Figs. 3B, 3C and 3D illustrate nanostructures provided with the narrow titanium-containing wires arranged in narrow pores of a porous alumina.
Fig. 4 conceptually illustrates the outline of a reactor for heat treatment used in the formation of narrow titanium-containing wires.
Fig. 5 conceptually illustrates the outline of an anodizing apparatus.
Fig. 6 conceptually illustrates porous alumina.
Fig. 7 is a schematic cross-sectional view illustrating an electron-emitting device according to an embodiment of the present invention.

### DESCRIPTION OF THE PREFERRED EMBODIMENTS

The embodiments of the present invention will hereinafter be described specifically.

### [Constitution of a narrow titanium-containing wire and a nanostructure to which the narrow titanium-containing wire is applied]

According to the present invention, the narrow titanium-containing wire and the nanostructure to which the narrow titanium-containing wire is applied are produced by forming a porous layer having narrow pores on a substrate having a titanium-containing surface and forming narrow titanium-containing wires in the respective narrow pores by carrying out a heat treatment under a specific atmosphere.

Figs. 3A, 3B, 3C and 3D conceptually illustrate examples of the nanostructure provided with the narrow titanium-containing wire. Fig. 3A illustrates a nanostructure composed of a substrate 10 having a layer 11 which constitutes a titanium-containing surface formed thereon, and the narrow titanium-containing wires 15 arranged in a specific direction (the substantially vertical direction) to the surface. Fig. 3B illustrates a nanostructure composed of a substrate 10 having a layer 11 which constitutes a titanium-containing surface formed thereon, a porous layer (porous alumina) 13 which has narrow pores 14 extending vertically to the surface provided on the surface, and the narrow titanium-containing wires 15 being arranged in the respective narrow pores 14.

The narrow titanium-containing wires 15 are formed of a metal, semiconductor or insulator comprising titanium as a main component, for example, any of titanium, titanium alloys including titanium-iron and titanium-aluminum, and optional titanium compounds such as titanium oxide, titanium hydride, titanium nitride and titanium carbide. The diameter (thickness) of the narrow titanium-containing wire 15 is generally within a range of from 1 nm to 2 µm, and the length thereof is generally within a range of from 10 nm to 100 µm.
Since the form of the narrow titanium-containing wire 15 is influenced by the form of the narrow pore of the porous layer to some extent, the pore diameter of the porous layer, an interval between the narrow pores, and the like are geometrically controlled, whereby the diameter and the like of the narrow titanium-containing wire can be controlled to some extent, and the growing direction of the narrow wire can also be controlled so as to extend vertically to the surface of the substrate by way of example.

Further, the narrow titanium-containing wire can be provided as a whisker crystal under special production conditions. Such conditions will be described subsequently.

As the porous layer formed on the titanium-containing surface at the structure illustrated in Fig. 3B, may be used porous alumina, zeolite, porous silicon, a mask formed by a photolithographic method, or the like. In particular, the porous alumina is desirable because it has linear narrow pores at regular intervals, so that narrow titanium-containing wires excellent in linearity can be formed at regular intervals, and moreover a nanostructure provided with the narrow titanium-containing wires 15 arranged at regular intervals in a specific direction (for example, the substantially vertical direction to the surface of the substrate) can be provided.

The structure of the porous alumina is illustrated in Fig. 6. The porous alumina 13 is composed mainly of Al and O, and many cylindrical and linear narrow pores 14 thereof are arranged substantially vertically to the surface of an aluminum film (plate) 601. The respective narrow pores are arranged at substantially regular intervals in parallel with one another. The narrow pores tend to be arranged in the form like a triangular lattice as illustrated in Fig. 6. The diameter 2r of the narrow pore is about 5 nm to 500 nm, and the interval 2R between the narrow pores is about 10 nm to 500 nm. The pore diameter and interval may be controlled to some extent by various process conditions such as the concentration and temperature of an electrolyte used in anodization, a method of applying anodizing voltage, anodizing voltage and time, and conditions of a subsequent pore widening treatment. In other words, the pore diameter and interval can be controlled, thereby controlling the diameter (thickness) of the narrow titanium-containing wire in a certain degree within the above range, for example, 300 nm or smaller in diameter.

In the nanostructure illustrated in Fig. 3B, the narrow titanium-containing wire 15 projects from the surface of the narrow pore. However, as illustrated in Fig. 3C, the growth of the narrow wire may also be stopped in the interior of the narrow pore to utilize it.

In Figs. 3B and 3C, the diameter of titanium-containing wire 15 is thinner than the diameter of the narrow pore 14 of anodic porous alumina. On the other hand, as illustrated in Fig. 3D, the diameter of titanium-containing wire 15 may be the same as the diameter of the narrow pore 14.

### [Production process of the narrow titanium-containing wire and the nanostructure to which the narrow titanium-containing wire is applied]

The narrow titanium-containing wire and the nanostructure to which the narrow titanium-containing wire is applied are preferably produced by a process comprising steps of providing a structure comprising a substrate having a titanium-containing surface and a porous layer containing narrow pores (Step 1); and forming narrow titanium-containing wires in the respective narrow pores by carrying out a heat treatment of the structure (Step 2).

The production process of the narrow titanium-containing wire and the nanostructure to which the narrow titanium-containing wire is applied will hereinafter be described in order with reference to Figs. 2A to 2D.

In Figs. 2A to 2D, reference numeral 10 indicates a substrate, 15 is a narrow titanium-containing wire, 11 is a titanium-containing film, 12 is an aluminum-containing film, 13 is a porous layer (porous alumina), 14 is a narrow pore (nanohole), and 15 is a narrow titanium-containing wire.

### Step 1: (Provision of the structure provided with the porous layer containing narrow pores on the substrate 10)

No particular limitation is imposed on the substrate 10 having the titanium-containing surface so far as it contains titanium on the surface. Examples thereof include plates of titanium or an alloy thereof, and substrates composed of any of various kinds of bases 16 such as quartz glass and Si and a Ti-containing film 11 formed on the base as illustrated in Fig. 2A.

The Ti-containing film 11 can be formed by one of optional film forming methods including resistance heating deposition, EB deposition, sputtering, CVD and plating.

The porous layer is preferably porous alumina which can be formed by an easy production process and contains narrow pores linear and high in aspect ratio. A process for forming the porous alumina as a porous layer will hereinafter be described.

### Step 1a: (Formation of the Al-containing film on the substrate)

The Al-containing film 12 illustrated in Fig. 2B can be formed by one of optional film forming methods including resistance heating deposition, EB deposition, sputtering, CVD and plating.

### Step 1b: (Anodizing step)

The Al-containing film 12 is subsequently anodized, thereby forming porous alumina 13 on the substrate (see Fig. 2C). The outline of an anodizing apparatus usable in this step is illustrated in Fig. 5.

In Fig. 5, reference numeral 50 indicates a thermostatic bath, 51 is a reaction vessel, 52 is a sample with an Al-containing film 12 formed on a substrate 10 having a Ti-containing surface, 53 is a Pt cathode, 54 is an electrolyte, 56 is a power source for applying anodizing voltage, and 55 is an ammeter for measuring an anodizing current (Ia). Besides, a computer (not illustrated) for automatically controlling and measuring the voltage and current, and the like are incorporated. The sample 52 and the cathode 53 are arranged in the electrolyte 54 the temperature of which is kept constant by the thermostatic bath 50. Voltage is applied between the sample 52 and the cathode 53 from the power source 56 to conduct the anodization.

Examples of the electrolyte used in the anodization include solutions of oxalic acid, phosphoric acid, sulfuric acid and chromic acid. Various conditions such as anodizing voltage and temperature may be suitably set according to a nanostructure to be produced.

In the anodizing step, the Al-containing film 12 is anodized over the entire film thickness. The anodization proceeds from the surface of the Al-containing film. When the anodization reaches the surface of the substrate 10, a change in the anodizing current is observed. Therefore, this change can be detected to judge whether the anodization is completed. For example, when a substrate with a Ti-containing film provided on an optional base is used, whether the application of the anodizing voltage is completed can be judged by a reduction in the anodizing current. After the anodizing treatment, the pore diameter of narrow pores can be suitably widened by a pore-widening treatment in which the treated substrate is immersed in an acid solution (for example, a phosphoric acid solution). The pore diameter can be controlled by the concentration of the solution, and treating time and temperature.

### Step 2: (Formation of the narrow titanium-containing wires in the narrow pores by a heat treatment)

The structure having the titanium-containing surface, on which the porous layer has been formed, is placed in a reaction vessel and subjected to a heat treatment under a specific atmosphere, whereby titanium present at the bottom of the narrow pores can be reacted with the atmosphere to form narrow titanium-containing wires 15 which is a reaction product of titanium and the atmosphere in the respective narrow pores of the porous layer (see Fig. 2D).

The reactor for conducting the heat treatment is described with reference to Fig. 4. In Fig. 4, reference numeral 41 indicates a reaction vessel, 42 is a sample (substrate), and 43 is an infrared absorbing plate which also assumes the part of a sample holder. Reference numeral 44 designates a pipe for introducing a gas such as hydrogen or oxygen, which is preferably arranged in such a manner that the concentration of the gas becomes uniform in the vicinity of the substrate. Reference numeral 46 indicates a gas discharging line connected to a turbo-molecular pump or rotary pump. Reference numeral 47 designates an infrared lamp for heating the base, and 48 is a condenser mirror for focusing infrared rays with good efficiency to the infrared absorbing plate. 49 is a window capable of transmitting the infrared rays. Besides, a vacuum gauge for monitoring the pressure within the reaction vessel and a thermocouple for measuring the temperature of the substrate (both, not illustrated) are incorporated. It goes without saying that besides the above-described apparatus, an electric furnace type apparatus which heats the whole structure from the outside may also be used without any particular problem.

The atmosphere and temperature used in the heat treatment are suitably set according to the material and form of a narrow titanium-containing wire to be produced. For example, when hydrogen, oxygen, nitrogen or a hydrocarbon is introduced as the atmosphere, a narrow wire correspondingly composed of titanium hydride, titanium oxide, titanium nitride or titanium carbide can be produced. Besides, materials used in the chemical vapor phase epitaxy, such as SiH₄, B₂H₅, PH₃, Al(C₂H₅)₃ and Fe(CO)₅, may also be used to form narrow wires containing titanium compounds such as titanium silicide, titanium boride, titanium phosphide, aluminum-titanium alloy and iron-titanium alloy, respectively. In particular, when a narrow wire composed of titanium oxide is produced, the heat treatment is conducted at a temperature ranging from 500°C to 900°C under an atmosphere containing at least 1 Pa of water vapor, whereby a narrow wire in the form of whisker can be formed. At this time, it is preferred that hydrogen is mixed into the atmosphere because the growth of the wire is accelerated. In general, whisker is a crystal grown in the form of a needle and has scarcely dislocation, and techniques such as deposition from a solution, decomposition of a compound and reduction of, for example, a halide with hydrogen have been known as the production methods thereof. The titanium oxide whisker according to the present invention is considered to be grown by an oxidation reaction with the water vapor and a reduction reaction with hydrogen (or heat).

Such a narrow titanium oxide wire having excellent crystallinity can be expected to have good electrical properties and electron-emitting properties as a semiconductor.

According to the process described above, the nanostructure illustrated in Fig. 3B, in which the narrow titanium-containing wires are present in the respective narrow pores of the porous layer, the narrow pores extending vertically to the Ti-containing surface, can be formed.

The porous layer 13 having the narrow pores, in which the narrow wires are present, of the structure thus obtained is removed by etching, thereby obtaining a nanostructure provided with the narrow Ti-containing wires on the Ti-containing surface of the substrate, the narrow wires extending vertically to the surface as illustrated in Fig. 3A.

Only the narrow wires are separated from the nanostructure illustrated in Fig 3A or 3B, whereby narrow wires having an extremely fine and even thickness and excellent linearity can be obtained.

The nanostructure obtained in the above-described manner can also be made to an electron-emitting device by arranging a counter electrode 701 in an opposing relation to the titanium-containing surface 11 in vacuum as illustrated in Fig. 7 and constructing them in such a manner that a potential may be applied between the titanium-containing surface 11 and the counter electrode 701. Since most of the narrow wires in the nanostructure used in this device extend in the direction substantially vertical to the surface, the device can be expected to emit electrons efficiently and stably.

The present invention will hereinafter be described in detail by the following Examples with reference to the drawings. However, the present invention is not limited to these examples.

### Example 1:

This example describes the production of a narrow titanium oxide wires and a nanostructure provided with the narrow titanium oxide wires.

The production process of the narrow titanium-containing wire and the nanostructure, to which the narrow wire is applied, according to the present invention is described in order with reference to Figs. 2A to 2D.

### Step 1:

In this example, a quartz base was used as a base 16. After the base was thoroughly washed with an organic solvent and purified water, a Ti film 11 having a thickness of 1 µm was formed on the base by sputtering to provide a substrate 10 (see Fig. 2A).

### Step 1a:

An Al film having a thickness of 1 µm was further formed as an Al-containing film 12 on the substrate 10 by sputtering (see Fig. 2B).

### Step 1b:

The Al-containing film 12 was subsequently subjected to an anodizing treatment using an anodizing apparatus illustrated in Fig. 5 (see Fig. 2C). A 0.3 M oxalic acid was used as an acid electrolyte, and kept at 17°C in a thermostatic bath. Anodizing voltage and treating time were set to DC 40 V and 10 minutes, respectively. In the course of the anodization process, i.e., after about 8 minutes, the anodization reached the surface (Ti film) of the substrate, and so reduction in the anodizing current was observed.

After the anodizing treatment, the diameter of narrow pores of the porous layer thus obtained was controlled by immersing the treated substrate in a 5 wt% phosphoric acid solution for 45 minutes as a pore-widening treatment. After the treatment, the substrate thus treated was washed with purified water and isopropyl alcohol.

### Step 2: (heat treating step)

The structure on the substrate of which the porous alumina had been formed was subsequently subjected to a heat treatment in a mixed atmosphere of water vapor, hydrogen and helium in accordance with the following process, thereby forming narrow titanium oxide wires. Namely, the structure was placed in a reaction vessel illustrated in Fig. 4. Hydrogen gas diluted to 1/50 with helium, passed through purified water kept at 5°C with bubbling was introduced at a flow rate of 50 sccm through a gas introducing pipe 44, while keeping the pressure within the reaction vessel at 1,000 Pa. An infrared lamp was then lit to heat the structure at 700°C for 1 hour, thereby heat-treating the structure. After the infrared lamp was put off, and the temperature of the structure was returned to room temperature, the feed of the gas was stopped to take the structure out in the air.

### Evaluation: (Observation of the structure)

The surface and section of the structure taken out were observed through an FE-SEM (field emission-scanning electron microscope).

### Result:

As illustrated in Fig. 3B, the porous alumina was formed with narrow pores having a diameter of about 60 nm and extending vertically to the surface of the Ti-containing film 11, the narrow pores being arranged at substantially regular intervals of about 100 nm in parallel with one another, and a large number of narrow wires grew within the respective narrow pores and from the interior of the narrow pores toward the outside. Each narrow titanium-containing wire grew from the surface of the substrate in the direction substantially vertical to the surface in accordance with the shape of the narrow pore, and had a diameter of about 40 to 60 nm and a length of several hundreds nanometers to several micrometers.

Further, the narrow wire was identified as being composed mainly of titanium by EDAX (energy non-dispersive X-ray diffraction analyzer). The X-ray diffraction of the narrow wire revealed that rutile type titanium oxide was present.

When the narrow titanium-containing wires formed in the narrow pores were separated from the substrate to observe them through a microscope at a high magnification, those in the form like a strand as illustrated in Fig. 1A, those in the form like a column as illustrated in Fig. 1B, those in the form like a column the thickness of which successively varied as illustrated in Fig. 1C, and those in the form with a plurality of columns united as illustrated in Fig. 1D were observed. Among those illustrated in Figs. 1B, 1C and 1D, those having an edge form corresponding to crystal face were included. They were considered to have undergone crystal growth, i.e., whisker growth.

### Example 2:

This example describes control of the diameter of a narrow titanium-containing wire by controlling the pore diameter of porous alumina.

Structures having porous alumina with the pore diameter thereof varied were provided in the same manner as in Example 1 except that anodizing voltage was set to 50 V, and the pore-widening treatment was conducted for varied periods of time of 0 minute, 15 minutes, 30 minutes, 45 minutes and 60 minutes. The typical pore diameters of the structures were 10 nm, 25 nm, 40 nm, 60 nm and 80 nm, respectively. These structures were then subjected to a heat treatment.
The heat treatment step was conducted in accordance with the step in Example 1.

As a result, the diameters of narrow titanium-containing wires formed in the narrow pores of the respective structures were influenced by the respective pore diameters, and so the structure having a greater pore diameter tended to have narrow wires having a greater diameter. Namely, each narrow titanium-containing wire was influenced by the form of the narrow pore to grow. Specifically, the average diameters of the respective narrow titanium-containing wires were 8 nm, 20 nm, 30 nm, 50 nm and 70 nm, respectively.

### Example 3:

This example describes control of the length of a narrow titanium-containing wire by controlling the conditions of a heat treatment.

Five structures having porous alumina on their substrates were provided in the same manner as in Example 1 except that the pore-widening treatment was conducted for 45 minutes. These structures were heat-treated in the same manner as in Example 1 except that the temperature of the heat treatment was varied to 600°C, 650°C, 700°C, 750°C and 800°C, respectively.

The nanostructures thus obtained were observed in the same manner as in Example 1. As a result, the observation by the FE-SEM revealed that in the nanostructure obtained by the heat treatment at 600°C, the growth of many narrow titanium-containing wires stopped midway in the narrow pore as illustrated in Fig. 3C. As the temperature of the heat treatment was raised higher, the narrow titanium-containing wire tended to become longer. The heat treatment at 700°C resulted in finding a number of narrow titanium-containing wires projected from the tops of the narrow pores as illustrated in Fig. 3B. In the heat treatment at 800°C, the diameters of titanium-containing wires were about 60nm and as same as the diameters of the narrow pores as illustrated in Fig. 3D.

### Example 4:

This example describes the formation of a nanostructure illustrated in Fig. 3A.

In this example, a nanostructure illustrated in Fig. 3B was produced in the same manner as in Example 1, and the porous alumina 13 thereof was then removed by etching with phosphoric acid.

In the nanostructure according to this example, as illustrated in Fig. 3A, narrow titanium-containing wires having a diameter of about 40 to 60 nm grew at intervals of about 100 nm from the surface of the substrate in the direction substantially vertical to the surface.

### Example 5:

This example describes the production of a narrow titanium oxide wire and a nanostructure provided with the narrow titanium oxide wire. This example followed Example 1 except for Step 2.

In Step 2 of this example, oxygen gas was introduced at a flow rate of 10 sccm into the reaction vessel, while keeping the pressure within the reaction vessel at 100 Pa. The structure was heated at 500°C for 1 hour, thereby heat-treating the structure.

Such narrow wires and nanostructure as illustrated in Fig. 3B were confirmed by FE-SEM. Further, the X-ray diffraction of the narrow wire revealed that anatase type titanium oxide was present.

The nanostructure according to this example was placed in an aqueous methanol solution (methanol:water = 1:6) and the whole light exposure by a high pressure mercury lamp was conducted. As a result, hydrogen was detected, and so it was confirmed that the nanostructure according to this example has a photocatalytic activity.

### Example 6:

This example describes the production of a narrow titanium carbide wire and a nanostructure provided with the narrow titanium carbide wire. This example followed Example 1 except for Step 2.

In Step 2 of this example, ethylene gas was introduced at a flow rate of 50 sccm into the reaction vessel, while keeping the pressure within the reaction vessel at 1,000 Pa. The structure was heated at 900°C for 1 hour, thereby heat-treating the structure.

Such narrow wires and nanostructure as illustrated in Fig. 3B were confirmed by FE-SEM. Further, the X-ray diffraction of the narrow wire revealed that titanium carbide was present.

The nanostructure according to this example and an anode having a fluorescent substance were arranged in opposition to each other at an interval of 1 mm in a vacuum device, and voltage of 1 kV was applied between the substrate and the anode. As a result, an electron emission current was observed together with emission of fluorescence from the fluorescent substance. This proved that the nanostructure according to this example could function as a good electron emitter.

As described above, the respective embodiments of the present invention can bring about, for example, the following effects.
(1) A narrow titanium-containing wire having a diameter of several tens nanometers to several hundreds nanometers can be produced with ease.
(2) A narrow titanium-containing wire having excellent linearity can be produced. In particular, titanium oxide whisker having excellent crystallinity can be obtained.
(3) A nanostructure comprising titanium as a main material can be obtained.
(4) A nanostructure provided with narrow titanium-containing wires having a specific directional property and a uniform diameter arranged at regular intervals on a substrate can be obtained.
(5) A high-performance electron-emitting device capable of emitting electrons in a greater amount can be obtained.

## Claims

1. A process for producing a structure having narrow titanium-containing wires (15), comprising steps of:
(i) providing a structure comprising a substrate (10) having a titanium-containing surface (11) and thereon a porous layer (13) having narrow pores (14) reaching said titanium-containing surface; and
(ii) forming narrow titanium-containing wires (15), projecting from said titanium-containing surface, into the respective narrow pores (14), by heat treatment under a specific atmosphere of the structure provided in step (i).

2. A process according to claim 1, wherein step (i) comprises sub-steps of:
forming an aluminum-containing film (12) on the substrate, and
anodically oxidizing the aluminum-containing film for providing said porous layer (13).

3. A process according to claim 1, wherein step (ii) comprises a sub-step of conducting the heat-treatment of the structure at a temperature ranging from 500°C to 900°C under an atmosphere containing water vapour of at least 1 Pa.

4. A process according to claim 1, wherein step (ii) comprises a sub-step of conducting the heat-treatment of the structure at a temperature ranging from 500°C to 900°C under an atmosphere containing water vapour of at least 1 Pa and hydrogen.

5. A process according to claim 1, wherein said specific atmosphere is an atmosphere containing a gas selected from the group consisting of hydrogen, oxygen, nitrogen, a hydrocarbon, SiH₄, B₂H₅, PH₃, Al(C₂H₅)₃ and Fe(CO)₅.

6. A process according to claim 1, wherein in step (ii) said titanium-containing wires are formed by a reaction of said surface with the gas of said atmosphere.

7. A process according to claim 1, wherein in step (ii) said titanium-containing wires are formed to have a diameter smaller than the diameter of said pores.

8. A process according to claim 1, further comprising a step of removing said porous layer after step (ii).

9. A process according to claim 1, wherein the diameter of said narrow titanium-containing wires (15) is within the range of 1 nm to 2 µm.

10. A process of producing narrow titanium-containing wires comprising steps (i) and (ii) of the process according to claim 1, and further comprising a step of separating only said titanium-containing wires from said structure after step (ii).

11. A structure comprising a substrate (10) having a titanium-containing surface (11), and narrow titanium-containing wires (15) projecting from said titanium-containing surface, in a direction substantially vertical to the surface.

12. A structure according to claim 11, wherein the narrow wires (15) are present in respective narrow pores (14) of a porous layer (13) provided on the surface, the narrow pores (14) extending in the direction vertical to the surface.

13. A structure according to claim 12, wherein the narrow wires (15) have a diameter of 300 nm or smaller.

14. A structure according to claim 12, wherein the narrow wires (15) contain at least one compound selected from the group consisting of titanium hydride, titanium oxide, titanium nitride and titanium carbide.

15. A structure according to claim 12, wherein the narrow wires (15) contain at least one compound selected from the group consisting of titanium silicide, titanium boride, titanium phosphide, aluminum-titanium alloy and iron-titanium alloy.

16. A structure according to claim 12, wherein the porous layer (13) is an anodically oxidized film.

17. A structure according to claim 16, wherein the porous layer (13) is an anodically oxidized film containing aluminum.

18. A structure according to claim 12, wherein each narrow wire (15) is a titanium oxide whisker.

19. A structure according to claim 11, wherein said titanium-containing wires are formed in respective pores (14) of a porous region (13) formed on said substrate, and the diameter of said titanium-containing wires (15) is smaller than the diameter of said pores (14).

20. A structure according to claim 11, wherein said surface comprises at least one of titanium or a titanium alloy, and the wires comprise at least one of titanium hydride, titanium oxide, titanium nitride, titanium carbide, titanium silicide, titanium boride or titanium phosphide.

21. A structure according to claim 11, wherein the diameter of said narrow titanium-containing wires is within the range of 1 nm to 2 µm.

22. A structure according to claim 12, wherein said wires project beyond the surface of the porous layer further from said titanium-containing surface.

23. An electron-emitting device comprising a structure, which comprises a substrate (10) having a titanium-containing surface (11), a porous layer (13) thereon having narrow pores (14) reaching said titanium-containing surface, and narrow titanium-containing wires (15), projecting from said titanium-containing surface respectively formed in the narrow pores (14); a counter electrode (701) arranged in an opposing relation to the titanium-containing surface (11); and a means for applying a potential between the titanium-containing surface (11) and the counter electrode (701).

## Patentansprüche

1. Verfahren zur Herstellung einer Struktur mit schmalen, Titan enthaltenden Drähten (15), welches die Schritte umfaßt:
(i) Bereitstellen einer Struktur, welche ein Substrat (10) mit einer Titan enthaltenden Oberfläche (11) und darauf einer porösen Schicht (13) mit schmalen Poren (14), welche die Titan enthaltende Oberfläche erreichen, aufweist; und
(ii) Bilden schmaler Titan enthaltender Drähte (15), welche von der Titan enthaltenden Oberfläche in die entsprechenden schmalen Poren (14) hinein hervorragen, durch Wärmebehandlung der in Schritt (i) bereitgestellten Struktur in einer spezifischen Atmosphäre.

2. Verfahren nach Anspruch 1, wobei Schritt (i) die Unterschritte umfaßt:
Bilden eines Aluminium enthaltenden Films (12) auf dem Substrat, und
anodisches Oxidieren des Aluminium enthaltenden Films zum Bereitstellen der porösen Schicht (13).

3. Verfahren nach Anspruch 1, wobei Schritt (ii) einen Unterschritt des Durchführens der Wärmebehandlung der Struktur bei einer Temperatur in einem Bereich von 500°C bis 900°C unter einer Atmosphäre, welche Wasserdampf von mindestens 1 Pa enthält, umfaßt.

4. Verfahren nach Anspruch 1, wobei Schritt (ii) einen Unterschritt des Durchführens der Wärmebehandlung und der Struktur bei einer Temperatur in einem Bereich von 500°C bis 900°C unter einer Atmosphäre, welche Wasserdampf von mindestens 1 Pa und Wasserstoff enthält, umfaßt.

5. Verfahren nach Anspruch 1, wobei die spezifische Atmosphäre eine Atmosphäre ist, welche ein Gas enthält, das aus der Gruppe ausgewählt wurde, die aus Wasserstoff, Sauerstoff, Stickstoff, einem Kohlenwasserstoff, SiH₄, B₂H₅, PH₃, Al(C₂H₅)₃ und Fe(CO)₅ besteht.

6. Verfahren nach Anspruch 1, wobei in Schritt (ii) die Titan enthaltenden Drähte durch eine Reaktion der Oberfläche mit dem Gas der Atmosphäre gebildet werden.

7. Verfahren nach Anspruch 1, wobei in Schritt (ii) die Titan enthaltenden Drähte mit einem Durchmesser kleiner als der Durchmesser der Poren gebildet werden.

8. Verfahren nach Anspruch 1, welches ferner einen Schritt des Entfernens der porösen Schicht nach Schritt (ii) umfaßt.

9. Verfahren nach Anspruch 1, wobei der Durchmesser der schmalen, Titan enthaltenden Drähte (15) in dem Bereich von 1 nm bis 2 µm liegt.

10. Verfahren zur Herstellung schmaler Titan enthaltender Drähte, welches die Schritte (i) und (ii) des Verfahrens nach Anspruch 1 umfaßt, und ferner einen Schritts des Abtrennens nur der Titan enthaltenden Drähte von der Struktur nach Schritt (ii) umfaßt.

11. Struktur, welche ein Substrat (10) mit einer Titan enthaltenden Oberfläche (11) und schmale Titan enthaltende Drähte (15) umfaßt, welche von der Titan enthaltenden Oberfläche in einer Richtung im Wesentlichen vertikal zu der Oberfläche herausragen.

12. Struktur nach Anspruch 11, wobei die schmalen Drähte (15) in entsprechenden schmalen Poren (14) einer auf der Oberfläche bereitgestellten porösen Schicht (13) vorhanden sind, wobei sich die schmalen Poren (14) in der Richtung vertikal zu der Oberfläche erstrecken.

13. Struktur nach Anspruch 12, wobei die schmalen Drähte (15) einen Durchmesser von 300 nm oder kleiner aufweisen.

14. Struktur nach Anspruch 12, wobei die schmalen Drähte (15) mindestens eine Verbindung enthalten, welche aus der Gruppe ausgewählt wurde, die aus Titanhydrid, Titanoxid, Titannitrid und Titancarbid besteht.

15. Struktur nach Anspruch 12, wobei die schmalen Drähte (15) mindestens eine Verbindung enthalten, welche aus der Gruppe ausgewählt wurde, die aus Titansilicid, Titanborid, Titanphosphid, Aluminium-Titan-Legierung und Eisen-Titan-Legierung besteht.

16. Struktur nach Anspruch 12, wobei die poröse Schicht (13) ein anodisch oxidierter Film ist.

17. Struktur nach Anspruch 16, wobei die poröse Schicht (13) ein Aluminium enthaltender anodisch oxidierter Film ist.

18. Struktur nach Anspruch 12, wobei jeder schmale Draht (15) ein Titanoxid-Whisker ist.

19. Struktur nach Anspruch 12, wobei die Titan enthaltenden Drähte in entsprechenden Poren (14) eines auf dem Substrat gebildeten porösen Bereichs (13) gebildet sind, und der Durchmesser der Titan enthaltenden Drähte (15) kleiner ist als der Durchmesser der Poren (14).

20. Struktur nach Anspruch 11, wobei die Oberfläche mindestens Titan oder eine Titanlegierung umfaßt, und die Drähte mindestens eine Verbindung von Titanhydrid, Titanoxid, Titannitrid, Titancarbid, Titansilicid, Titanborid oder Titanphosphid umfassen.

21. Struktur nach Anspruch 11, wobei der Durchmesser der schmalen Titan enthaltenden Drähte in einem Bereich von 1 nm bis 2 µm liegt.

22. Struktur nach Anspruch 12, wobei die Drähte hinter der Oberfläche der porösen Schicht weiter von der Titan enthaltenden Oberfläche hervorragen.

23. Elektronen emittierende Vorrichtung, die eine Struktur umfaßt, welche ein Substrat (10) mit einer Titan enthaltenden Oberfläche (11), eine poröse Schicht (13) darauf mit schmalen Poren (14), welche die Titan enthaltende Oberfläche erreichen, und schmale Titan enthaltende Drähte (15), welche von der Titan enthaltenden Oberfläche hervorragen und jeweils in den schmalen Poren (14) gebildet sind; eine Gegenelektrode (701), welche in einer gegenüberstehenden Beziehung zu der Titan enthaltenden Oberfläche (11) angeordnet ist; und eine Einrichtung zum Anlegen eines Potentials zwischen der Titan enthaltenden Oberfläche (11) und der Gegenelektrode (701) umfaßt.

## Revendications

1. Procédé pour la production d'une structure ayant des fils fins (15) contenant du titane, comprenant les étapes qui consistent :
(i) à utiliser une structure comportant un substrat (10) ayant une surface (11) contenant du titane et portant une couche poreuse (13) ayant des pores étroits (14) atteignant ladite surface contenant du titane ; et
(ii) à former des fils fins (15) contenant du titane, faisant saillie de ladite surface contenant du titane, dans les pores étroits respectifs (14), par un traitement thermique sous une atmosphère spécifique de la structure produite dans l'étape (i).

2. Procédé selon la revendication 1, dans lequel l'étape (i) comprend les sous-étapes qui consistent :
à former un film (12) contenant de l'aluminium sur le substrat, et
à appliquer une oxydation anodique au film contenant de l'aluminium pour produire ladite couche poreuse (13).

3. Procédé selon la revendication 1, dans lequel l'étape (ii) comprend une sous-étape consistant à exécuter le traitement thermique de la structure à une température allant de 500°C à 900°C sous une atmosphère contenant de la vapeur d'eau à au moins 1 Pa.

4. Procédé selon la revendication 1, dans lequel l'étape (ii) comprend une sous-étape consistant à exécuter le traitement thermique de la structure à une température allant de 500°C à 900°C sous une atmosphère contenant de la vapeur d'eau à au moins 1 Pa et de l'hydrogène.

5. Procédé selon la revendication 1, dans lequel ladite atmosphère spécifique est une atmosphère contenant un gaz choisi dans le groupe consistant en l'hydrogène, l'oxygène, l'azote, un hydrocarbure, SiH₄, B₂H₅, PH₃, Al(C₂H₅)₃ et Fe(CO)₅.

6. Procédé selon la revendication 1, dans lequel, dans l'étape (ii), lesdits fils contenant du titane sont formés par une réaction de ladite surface avec le gaz de ladite atmosphère.

7. Procédé selon la revendication 1, dans lequel, dans l'étape (ii), lesdits fils contenant du titane sont formés de façon à avoir un diamètre inférieur au diamètre desdits pores.

8. Procédé selon la revendication 1, comprenant en outre une étape consistant à enlever ladite couche poreuse après l'étape (ii).

9. Procédé selon la revendication 1, dans lequel le diamètre desdits fils fins (15) contenant du titane est compris dans la plage de 1 nm à 2 µm.

10. Procédé de production de fils fins contenant du titane, comprenant les étapes (i) et (ii) du procédé selon la revendication 1, et comprenant en outre une étape consistant à séparer uniquement lesdits fils contenant du titane de ladite structure après l'étape (ii).

11. Structure comportant un substrat (10) ayant une surface (11) contenant du titane, et des fils fins (15) contenant du titane faisant saillie de ladite surface contenant du titane, dans une direction sensiblement perpendiculaire à la surface.

12. Structure selon la revendication 11, dans laquelle les fils fins (15) sont présents dans des pores étroits respectifs (14) d'une couche poreuse (13) située sur la surface, les pores étroits (14) s'étendant dans la direction perpendiculaire à la surface.

13. Structure selon la revendication 12, dans laquelle les fils fins (14) ont un diamètre de 300 nm ou moins.

14. Structure selon la revendication 12, dans laquelle les fils fins (15) contiennent au moins un composé choisi dans le groupe consistant en de l'hydrure de titane, de l'oxyde de titane, du nitrure de titane et du carbure de titane.

15. Structure selon la revendication 12, dans laquelle les fils fins (15) contiennent au moins un composé choisi dans le groupe consistant en du siliciure de titane, du borure de titane, du phosphure de titane, un alliage aluminium-titane et un alliage fer-titane.

16. Structure selon la revendication 12, dans laquelle la couche poreuse (13) est un film oxydé anodiquement.

17. Structure selon la revendication 16, dans laquelle la couche poreuse (13) est un film oxydé anodiquement contenant de l'aluminium.

18. Structure selon la revendication 12, dans laquelle chaque fil fin (15) est une trichite d'oxyde de titane.

19. Structure selon la revendication 11, dans laquelle lesdits fils contenant du titane sont formés dans des pores respectifs (14) d'une région poreuse (13) formée sur ledit substrat, et le diamètre desdits fils (15) contenant du titane est plus petit que le diamètre desdits pores (14).

20. Structure selon la revendication 11, dans laquelle ladite surface comprend au moins l'un du titane ou d'un alliage de titane, et les fils comprennent au moins l'un de l'hydrure de titane, de l'oxyde de titane, du nitrure de titane, du carbure de titane, du siliciure de titane, du borure de titane ou du phosphure de titane.

21. Structure selon la revendication 11, dans laquelle le diamètre desdits fils fins contenant du titane est compris dans la plage de 1 nm à 2 µm.

22. Structure selon la revendication 12, dans laquelle lesdits fils s'étendent depuis ladite surface contenant du titane en faisant saillie au-delà de la surface de la couche poreuse.

23. Dispositif d'émission d'électrons comportant une structure, qui comporte un substrat (10) ayant une surface (11) contenant du titane, une couche poreuse (13) sur cette surface ayant des pores étroits (14) atteignant ladite surface contenant du titane, et des fils fins (15) contenant du titane, faisant saillie de ladite surface contenant du titane et formés respectivement dans les pores étroits (14) ; une contre-électrode (701) agencée de façon à être opposée à la surface (11) contenant du titane ; et un moyen destiné à appliquer un potentiel entre la surface (11) contenant du titane et la contre-électrode (701).
